



US007541124B2

(12) **United States Patent**  
**Molaire et al.**

(10) **Patent No.:** **US 7,541,124 B2**  
(45) **Date of Patent:** **\*Jun. 2, 2009**

(54) **CONDENSATION POLYMER  
PHOTOCONDUCTIVE ELEMENTS**

(75) Inventors: **Michel F. Molaire**, Rochester, NY (US);  
**Wayne T. Ferrar**, Fairport, NY (US);  
**David S. Weiss**, Rochester, NY (US);  
**John C. Wilson**, Rochester, NY (US)

(73) Assignee: **Eastman Kodak Company**, Rochester, NY (US)

(\*) Notice: Subject to any disclaimer, the term of this patent is extended or adjusted under 35 U.S.C. 154(b) by 455 days.

This patent is subject to a terminal disclaimer.

(21) Appl. No.: **11/210,100**

(22) Filed: **Aug. 19, 2005**

(65) **Prior Publication Data**

US 2007/0042282 A1 Feb. 22, 2007

(51) **Int. Cl.**  
**G03G 5/14** (2006.01)

(52) **U.S. Cl.** ..... **430/64; 430/123.4**

(58) **Field of Classification Search** ..... **430/60,  
430/64, 65, 123.4**

See application file for complete search history.

(56) **References Cited**

U.S. PATENT DOCUMENTS

3,428,451 A 2/1969 Trevoy  
4,082,551 A 4/1978 Steklenski et al.

|              |         |                 |
|--------------|---------|-----------------|
| 4,971,873 A  | 11/1990 | Pavlisko et al. |
| 5,128,226 A  | 7/1992  | Hung            |
| 5,681,677 A  | 10/1997 | Bugner et al.   |
| 6,294,301 B1 | 9/2001  | Sorriero et al. |
| 6,451,956 B2 | 9/2002  | Sorriero et al. |
| 6,593,046 B2 | 7/2003  | Sorriero et al. |
| 6,866,977 B2 | 3/2005  | Sorriero et al. |

OTHER PUBLICATIONS

Japanese Patent Office English-language abstract describing JP 2003-330209, copyright 1998.\*

Japanese Patent Office English-language abstract describing JP 2003-327587, copyright 1998.\*

Michel Molair, "Photoconductive Element Having an Amorphous, Polymeric Barier Layer", filed as U.S. Appl. No. 10/888,172 on Jul. 9, 2004.

\* cited by examiner

*Primary Examiner*—Janis L Dote

(74) *Attorney, Agent, or Firm*—Carl F. Ruoff; Andrew J. Anderson

(57) **ABSTRACT**

The present invention relates to photoconductive elements having an electrically conductive support, an electrical barrier layer and, disposed over the barrier layer, a charge generation layer capable of generating positive charge carriers when exposed to actinic radiation. The electrical barrier layer, which restrains injection of positive charge carriers from the conductive support, comprises a crosslinker, a crosslinkable condensation polymer having as a repeating unit a planar, electron-deficient tetracarbonylbisimide group.

**13 Claims, 1 Drawing Sheet**



*FIG. 1*

## 1

CONDENSATION POLYMER  
PHOTOCONDUCTIVE ELEMENTS

## FIELD OF THE INVENTION

This invention relates to electrophotography. More particularly, it relates to polymers comprising a tetracarbonylbisimide group and to photoconductive elements that contain an electrical charge barrier layer comprised of said polymers.

## BACKGROUND OF THE INVENTION

Photoconductive elements useful, for example, in electro-photographic copiers and printers are composed of a conducting support having a photoconductive layer that is insulating in the dark but becomes conductive upon exposure to actinic radiation. To form images, the surface of the element is electrostatically and uniformly charged in the dark and then exposed to a pattern of actinic radiation. In areas where the photoconductive layer is irradiated, mobile charge carriers are generated which migrate to the surface and dissipate the surface charge. This leaves in non-irradiated areas a charge pattern known as a latent electrostatic image. The latent image can be developed, either on the surface on which it is formed or on another surface to which it is transferred, by application of a liquid or dry developer containing finely divided charged toner particles.

Photoconductive elements can comprise single or multiple active layers. Those with multiple active layers (also called multi-active elements) have at least one charge-generation layer and at least one n-type or p-type charge-transport layer. Under actinic radiation, the charge-generation layer generates mobile charge carriers and the charge-transport layer facilitates migration of the charge carriers to the surface of the element, where they dissipate the uniform electrostatic charge and form the latent electrostatic image.

Also useful in photoconductive elements are charge barrier layers, which are formed between the conductive layer and the charge generation layer to restrict undesired injection of charge carriers from the conductive layer. Various polymers are known for use in barrier layers of photoconductive elements. For example, Hung, U.S. Pat. No. 5,128,226, discloses a photoconductor element having an n-type charge transport layer and a barrier layer, the latter comprising a particular vinyl copolymer. Steklenski, et al. U.S. Pat. No. 4,082,551, refers to Trevoy U.S. Pat. No. 3,428,451, as disclosing a two-layer system that includes cellulose nitrate as an electrical barrier. Bugner et al. U.S. Pat. No. 5,681,677, discloses photoconductive elements having a barrier layer comprising certain polyester ionomers. Pavlisko et al., U.S. Pat. No. 4,971,873, discloses solvent-soluble polyimides as polymeric binders for photoconductor element layers, including charge transport layers and barrier layers.

Still further, a number of known barrier layer materials function satisfactorily only when coated in thin layers. As a consequence, irregularities in the coating surface, such as bumps or skips, can alter the electric field across the surface. This in turn can cause irregularities in the quality of images produced with the photoconductive element. One such image defect is caused by dielectric breakdowns due to film surface irregularities and/or non-uniform thickness. This defect is observed as toner density in areas where development should not occur, also known as breakdown.

The known barrier layer materials have certain drawbacks, especially when used with negatively charged elements having p-type charge transport layers. Such elements are referred to as p-type photoconductors. Thus, a negative surface charge

## 2

on the photoconductive element requires the barrier material to provide a high-energy barrier to the injection of positive charges (also known as holes) and to transport electrons under an applied electric field. Many known barrier layer materials are not sufficiently resistant to the injection of positive charges from the conductive support of the photoconductive element. Also, for many known barrier materials the mechanism of charge transport is ionic. This property allows for a relatively thick barrier layer for previously known barrier materials, and provides acceptable electrical properties at moderate to high relative humidity (RH) levels. Ambient humidity affects the water content of the barrier material and, hence, its ionic charge transport mechanism. Thus, at low RH levels the ability to transport charge in such materials decreases and negatively impacts film electrical properties. A need exists for charge barrier materials that transport charge by electronic as well as ionic mechanisms so that films are not substantially affected by humidity changes.

Condensation polymers of polyester-co-imides, polyesters-trionomer-co-imides, and polyamide-co-imides are all addressed in:

1. Sorriero et al. in U.S. Pat. No. 6,294,301.
2. Sorriero et al. in U. S. Pat. No. 6,451,956.
3. Sorriero et al. in U. S. Pat. No. 6,593,046.
4. Sorriero et al. in U. S. Pat. 6,866,977.
5. Molaire et al. in U. S. Pat. No. 7,267,915.

These polymers have as a repeating unit a planar, electron-deficient, tetracarbonylbisimide group that is in the polymer backbone. The polymers are either soluble in chlorinated solvents and chlorinated solvent-alcohol combinations, or they contain salts to achieve solubility in polar solvents. In all cases, care must be taken not to disrupt the layer with subsequent layers that are coated from solvents, as this may result in swelling of the electron transport layer, mixing with the layer, or dissolution of part or all of the polymer. Furthermore, salts can make the layer subject to unwanted ionic transport.

Japanese Kokai Tokkyo Koho 2003330209A to Canon includes polymerizable naphthalene bisimides among a number of polymerizable electron transport molecules. Some of the naphthalene bisimides contain acrylate functional groups, epoxy groups, and hydroxyl groups. The monomers are polymerized after they are coated onto an electrically conductive substrate. However this approach does not ensure the full incorporation of all of the monomers. Some of the functional groups would not react to form a film and could thus be extracted during the deposition of subsequent layers. This would result in a layer that was not the same composition as deposited before polymerization. Further, it would allow for the unwanted incorporation of the electron transport agent into the upper layers of the photoreceptor by contamination of the coating solutions. Thus the need remains for a well characterized electron transport polymer that can be coated and crosslinked completely to produce a layer that will transport electrons between layers of a photoreceptor without contaminating subsequent layers.

Japanese Kokai Tokkyo Koho 2003327587A to Canon describes the synthesis of naphthalene bisimide acrylate polymers. The polymers were coated from solution onto aluminum MYLAR™ and irradiated with an electron beam to harden the layer to form crack free films. Mobility measurements were made. The need exists to form an insoluble film from a polymer that can transport electrons and has active sites for crosslinking that result in a film that can be overcoated with subsequent layers to form a photoreceptor. The crosslinking should be done either thermally or with UV light.

Photoconductive elements typically are multi-layered structures wherein each layer, when it is coated or otherwise formed on a substrate, needs to have structural integrity and desirably a capacity to resist attack when a subsequent layer is coated on top of it or otherwise formed thereon. Such layers are typically solvent coated using a solution with a desired coating material dissolved or dispersed therein. This method requires that each layer of the element, as such layer is formed, should be capable of resisting attack by the coating solvent employed in the next coating step. A need exists for a negatively chargeable photoconductive element having a p-type photoconductor, and including an electrical barrier layer that can be coated from an aqueous or organic medium, that has good resistance to the injection of positive charges, can be sufficiently thick and uniform that minor surface irregularities do not substantially alter the field strength, and resists hole transport over a wide humidity range. Still further, a need exists for photoconductive elements wherein the barrier layer is substantially impervious to, or insoluble in, solvents used for coating other layers, e.g., charge generation layers, over the barrier layer.

Accordingly, a need exists for a negatively chargeable photoconductive element having a p-type photoconductor, and including an electrical barrier layer that can be coated from an aqueous or organic medium, that has good resistance to the injection of positive charges, can be sufficiently thick and uniform that minor surface irregularities do not substantially alter the field strength, and resists hole transport over a wide humidity range. Still further, a need exists for photoconductive elements wherein the barrier layer is substantially impervious to, or insoluble in, solvents used for coating other layers, e.g., charge generation layers, over the barrier layer.

Photoconductive elements comprising a photoconductive layer formed on a conductive support such as a film, belt or drum, with or without other layers such as a barrier layer, are also referred to herein, for brevity, as photoconductors.

#### PROBLEM TO BE SOLVED BY THE INVENTION

A need exists for a negatively chargeable photoconductive element having a p-type photoconductor, and including an electrical barrier layer that can be coated from an aqueous or organic medium, that has good resistance to the injection of positive charges, can be sufficiently thick and uniform that minor surface irregularities do not substantially alter the field strength, and resists hole injection and transport over a wide humidity range. Still further, a need exists for photoconductive elements wherein the barrier layer is substantially impervious to, or insoluble in, solvents used for coating other layers, e.g., charge generation layers, over the barrier layer.

#### SUMMARY OF THE INVENTION

The present invention relates to a photoconductive element comprising an electrically conductive support, an electrical barrier layer disposed over said electrically conductive support, and disposed over said barrier layer, a charge generation layer capable of generating positive charge carriers when exposed to actinic radiation, said barrier layer comprising condensation polymer with aromatic tetracarbonylbisimide groups and crosslinking sites.

The crosslinkable condensation polymer has covalently bonded as repeating units in the polymer chain, aromatic tetracarbonylbisimide groups of the formula:



5

10

15

20

25

30

35

40

45

50

55

60

65

wherein Ar represents a tetravalent aromatic group.

More specifically, the barrier layer polymer is a polyester-co-imide that contains an aromatic tetracarbonylbisimide group and has the formula:



where

x=mole fraction of tetracarbonylbisimide diacid residue in the diacid component of the monomer feed from 0-1 and

y=mole fraction of tetracarbonylbisimide glycol residue in the glycol component of the monomer feed from 0-1

such that  $x+(1-y)=0.1$  to 1.9.

Ar¹ and Ar²=a tetravalent aromatic group having from 6 to 20 carbon atoms and may be the same or different. Representative groups include:





where Z =



R<sup>1</sup>, R<sup>2</sup>, R<sup>3</sup>, and R<sup>4</sup>=alkylene and may be the same or different. Representative alkylene moieties include 1,3-propylene, 1,5-pentanediyi and 1,10-decanediyi.

R<sup>5</sup>=alkylene or arylene. Representative moieties include 1,4-cyclohexylene, 1,2-propylene, 1,4-phenylene, 1,3-phenylene, 5-t-butyl-1,3-phenylene, 2,6-naphthalene, vinylene, 1,1,3-trimethyl-3-(4-phenylene)-5-indanyl, 1,12-dodecanediyi, and the like.

R<sup>6</sup>=alkylene such as ethylene, 2,2-dimethyl-1,3-propylene, 1,2-propylene, 1,3-propylene, 1,4-butanediyi, 1,6-hexanediyi, 1,10-decanediyi, 1,4-cyclohexanedimethylene, 2,2'-oxydiethylene, polyoxyethylene, tetraoxyethylene, and the like,

or hydroxyl substituted alkylene such as 2-hydroxymethyl-1,3-propanediyi, 2-hydroxymethyl-2-ethyl-1,3-propanediyi, 2,2-bis(hydroxymethyl)-1,3-propanediyi, and the like.

#### ADVANTAGEOUS EFFECT OF THE INVENTION

The invention provides for a negatively chargeable photoconductive element having a p-type photoconductor, and including an electrical barrier polymer that has good resistance to the injection of positive charges, can be sufficiently thick and uniform that minor surface irregularities do not substantially alter the field strength, and resists hole transport over a wide humidity range. The barrier polymer is prepared from a condensation polymer having pendent planar, electron-deficient, tetracarbonylbisimide groups. This barrier polymer is substantially impervious to, or insoluble in, solvents used for coating other layers, e.g., charge generation layers, over the barrier polymer layer.

#### BRIEF DESCRIPTION OF THE DRAWINGS

FIG. 1 is a schematic cross section, not to scale, for one embodiment of a photoconductive element according to the invention.

#### DETAILED DESCRIPTION OF THE INVENTION

The invention has numerous advantages. As illustrated in FIG. 1, the invention provides an embodiment of a photoconductive element 10 of the invention comprises a flexible polymeric film support 11. On this support is coated an electrically conductive layer 12. Over the conductive layer 12 is coated a polymeric barrier layer 13, the composition of which is indicated above and described more fully hereinafter. Over the barrier layer 13 is coated a charge generation layer 14, and over the latter is coated a p-type charge transport layer 15. The p-type charge transport layer 15 is capable of transporting positive charge carriers generated by charge generation layer

14 in order to dissipate negative charges on the surface 16 of the photoconductive element 10.

The barrier and other layers of the photoconductive element are coated on an “electrically-conductive support,” by which is meant either a support material that is electrically-conductive itself or a support material comprising a non-conductive substrate, such as support 11 of the drawing, on which is coated a conductive layer 12, such as vacuum deposited or electroplated metals, such as nickel. The support can be fabricated in any suitable configuration, for example, as a sheet, a drum, or an endless belt. Examples of “electrically-conductive supports” are described in Bugner et al., U.S. Pat. No. 5,681,677, the teachings of which are incorporated herein by reference in their entirety.

The barrier layer composition can be applied to the electrically conductive substrate by coating the substrate with an aqueous dispersion or solution of the barrier layer polymer using, for example, well known coating techniques, such as knife coating, dip coating, spray coating, swirl coating, extrusion hopper coating, or the like. In addition to water, other solvents which are suitable are polar solvents, such as alcohols, like methanol, ethanol, propanol, isopropanol, and mixtures thereof. As indicated in the examples hereinafter, such polar solvents can also include ketones, such as acetone, methylethylketone, methyl isobutyl ketone, or mixtures thereof. After application to the conductive support, the so-coated substrate can be air dried. It should be understood, however, that, if desired, the barrier layer polymers can be coated as solutions or dispersions in organic solvents, or mixtures of such organic solvents and water, by solution coating techniques known in the art.

Typical solvents for solvent coating a photoconductive charge generation layer over a charge barrier layer are disclosed, for example, in Bugner et al., U.S. Pat. No. 5,681,677; Molaire et al., U.S. Pat. No. 5,733,695; and Molaire et al., U.S. Pat. No. 5,614,342, the teachings of which are all incorporated herein by reference in their entirety. As these references indicate, the photoconductive material, e.g., a photoconductive pigment, is solvent coated by dispersing it in a binder polymer solution. Commonly used solvents for this purpose include chlorinated hydrocarbons, such as dichloromethane, as well as ketones and tetrahydrofuran. A problem with known barrier layer compositions is that such solvents for the coating of the photoconductive or charge generation layer will also dissolve or damage the barrier layer. An advantage of the barrier layer compositions of the invention is crosslinking sites are incorporated into the polymer. Because the barriers are crosslinked, they are not substantially dissolved or damaged by chlorinated hydrocarbons or the other commonly used solvents for coating photoconductor or charge generation layers, at the temperatures and for the time periods employed for coating such layers. This is achieved by using the end groups of the polymer to react with crosslinking agents, or through copolymerization with difunctional monomers that incorporate the functional groups that are available for reaction with a crosslinking agent. The crosslinked polymers are not substantially dissolved or damaged by chlorinated hydrocarbons or the other commonly used solvents for coating photoconductor or charge generation layers, at the temperatures and for the time periods employed for coating such layers.

There are many commercial crosslinking agents that will react when heated for a sufficient period of time with an active functional group of a polymer to form crosslinked networks. Some of the more common methods of thermal crosslinking are listed below.

- Dihydroxydioxane has been used to crosslink gelatin and polyvinylalcohol. Acid is needed to catalyze the reaction when amines are not present.
- PRIMIDSTM (Ems-Chemie AG in Domat/Switzerland) are  $\beta$ -hydroxyalkylamides that will react with organic acid moieties on polymers.
- CYMELTM crosslinking agents are highly methylated melamine-formaldehyde resins where the methoxymethyl group reacts with a hydroxy group on a polymer.
- Radical initiators such as benzoyl peroxide that will react at elevated temperatures with olefins to form covalent crosslinks.
- Blocked Isocyanate crosslinking agents are used to crosslink hydroxy compounds to form urethanes.
- Thiol-ene systems that operate by thermal or photo-crosslinking and are relatively insensitive to atmospheric oxygen.
- Diethyl malonate blocked isocyanates are a form of the blocked isocyanates that crosslinks using ester exchange. This differs from other isocyanate blocking chemistry in that the product of the crosslinking is an ester and an alcohol. Traditional blocked isocyanate crosslinkers are more likely to produce free isocyanates and amino compounds that could interfere with electron transport. The structure of the crosslinker known as Tri-zene BI 7963 from Baxenden Chemicals Limited, Paragon Works, Baxenden, Accrington, Lancashire BB5 2SL, England is represented as:



Various catalysts can also be added to the polymer and crosslinker. In particular, tin compounds such as dibutyltin dilaurate can be added in small amounts to improve the crosslinking reaction. Bismuth compounds are also known to catalyze the crosslinking, such as K-KAT XC-C227 from King Industries, Science Road, Norwalk, Conn. 06852.

References to crosslinking chemistry include:

- Wicks, D. A.; Wicks, Z. W. *Prog. Org. Coat.* 1999, 36, 148.  
 Wicks, D. A.; Wicks, Z. W. *Prog. Org. Coat.* 2001, 41, 1.  
 Maier, S.; Loontjens, T; Scholtens, B.; Mulhaupt, R.; *Macromolecules*, 2003, 36, 4727.  
 Jones, J. *Paint & Resin Times* 2002, April/May 1(3): 9-11.  
 Tabor, B. E.; Owers, R.; Janus, J. W.; *J. Photographic Science*, 1992, 40, 205.  
 Reddy, S. K.; Cramer, N. B.; Rydholm, A.; Anseth, K. S.; Bowman, C. N.; *Polymer Preprints* 2004, 45 (2), 65.

Webster, G., Ed. *Prepolymers & Reactive Diluents*, Volume 11 in *Chemistry & Technology of UV & EB Formulations for Coatings, Inks & Paints*.

The advantage of crosslinking the polyester-co-imide is that the cured polymer is insoluble in all solvents. Thus the polymer can be overcoated with any solvent system, without regard to the solubility of any subsequent layers of coating. This is a substantial advantage over previous bisimide polymers prepared by condensation polymerization, where the subsequent layers had to be coated from solvents that would not dissolve the barrier layer. Additionally, intermixing of the barrier layer with other layers can be minimized or eliminated by controlling the degree of crosslinking in the barrier layer.

For example, certain polyamides of the barrier layer polymers of the prior art were dissolved in mixtures of dichloromethane with a polar solvent such as methanol or ethanol. The polyamide barrier layers were "substantially insoluble" in chlorinated hydrocarbons and could be overcoated with solvents such as dichloromethane. However, that solvent could not also contain an alcohol as that would render the imide containing polyamide soluble and results in dissolution of the layer. The barrier layer polymers of the present invention are not limited by this restriction and can be overcoated with a wide variety of solvents, including the same solvent as the polymer was originally coated from. The examples could be coated from THF, cured, and overcoated with a THF solution of another polymer to deposit a layer such as a charge generation layer on the barrier layer. In a similar manner, the polyesterionomers-co-imides of the prior art employ polar solvents to deposit the electron transport barrier layer onto the substrate. Overcoating with subsequent layers is then limited to solvents that will not destroy the polymer or cause mixing with subsequent layers, and thus only non-polar solvents can be used to coat the subsequent layers. This can be a disadvantage as it limits the choice of compounds that can be overcoated onto the barrier layer. It also necessitates the use of organic solvents that are often not as environmentally desirable as polar solvents such as alcohols and water. Thus the crosslinked polyester-co-imides allow for a broader choice of coating solvents in the formulations of the photoreceptors.

The compositions of, the locations, and methods for forming the photoconductive charge generating layer, the charge transport layer, and other components of the photoconductive element of the invention are as described in Bugner et al. U.S. Pat. No. 5,681,677 cited above and incorporated herein by reference in its entirety.

A preferred conductive support for use in electrophotographic and laser copiers or printers is a seamless, flexible cylinder or belt of polymer material on which nickel can be electroplated or vacuum deposited. Other useful supports include belts or cylinders with layers of other metals, such as aluminum, stainless steel or copper, deposited thereon. Such conductive supports have important advantages but at least one drawback for which the barrier layer compositions of the present invention, and particularly certain preferred polyester-co-imide as described more fully hereinafter, provide a solution. The deposited nickel layers often bumps or other irregularities which, when the barrier layer is thin, can cause an irregular electric field strength across the surface and thus cause defects, electrical breakdown, or so-called black spots in the resulting image. Thus, irregularities on the electrically

conductive support make it desirable to have a barrier layer which can be coated at thicknesses which are adequate to smooth out this surface roughness. As an advantage over conventional barrier materials, the barrier materials of the present invention can be formed in relatively thick layers and still have desired electrophotographic properties. As a relatively thick layer, e.g., greater than 1 micron and, in more preferred embodiments, greater than 1.2 microns, preferably greater than about 2 microns, more preferably greater than about 3 microns, and most preferably greater than about 4 microns, the barrier layer of the invention can act as a smoothing layer and compensate for such surface irregularities. In particular, the preferred polyester-co-imides described below can be coated as a relatively thick barrier layer, in comparison to those elements in the prior art with good performance in an electrophotographic film element. In one embodiment of the invention, the barrier layer may have a thickness of between 0.5 and 3 micrometers.

We have found that although several crosslinking chemistries give satisfactory degrees of crosslinking of the bisimide films, the techniques that avoid acids and bases are the most satisfactory for polyester-co-bisimides that carry charge. One method of crosslinking that we have employed uses diethyl malonate blocked isocyanates. These are a form of the blocked isocyanates that crosslink using ester exchange. This differs from other isocyanate blocking chemistry in that the product of the crosslinking is an alcohol. Traditional blocked isocyanate crosslinkers unblock to form free isocyanates at curing temperatures. Residual isocyanates that do not form crosslinks may interfere with charge transport, or they may hydrolyze to form amines or some other more reactive species that could interfere with the charge transport of the polymers. In particular the crosslinking of the polymer below with a dimethylmalonate blocked isocyanates results in the formation of ethanol which is volatilized in the curing process.

The barrier layer polymer employed is a condensation polymer that contains as a repeating unit a planar, electron-deficient aromatic tetracarbonylbisimide group as defined above.

The barrier layer polymer is a polyester-co-imide that contains an aromatic tetracarbonylbisimide group and has the formula:



where

x=mole fraction of tetracarbonylbisimide diacid residue in the diacid component of the monomer feed from 0-1 and

y=mole fraction of tetracarbonylbisimide glycol residue in the glycol component of the monomer feed from 0-1

such that  $x+(1-y)=0.1$  to 1.9.

Ar<sup>1</sup> and Ar<sup>2</sup>=a tetravalent aromatic group having from 6 to 20 carbon atoms and may be the same or different. Representative groups include:



where Z =



R<sup>1</sup>, R<sup>2</sup>, R<sup>3</sup>, and R<sup>4</sup>=alkylene and may be the same or different. Representative alkylene moieties include 1,3-propylene, 1,5-pentanediyi and 1,10-decanediyi.

R<sup>5</sup>=alkylene or arylene. Representative moieties include 1,4-cyclohexylene, 1,2-propylene, 1,4-phenylene, 1,3-phenylene, 5-t-butyl-1,3-phenylene, 2,6-naphthalene, vinylene, 1,1,3-trimethyl-3-(4-phenylene)-5-indanyl, 1,12-dodecanediyi, and the like.

R<sup>6</sup>=alkylene such as ethylene, 2,2-dimethyl-1,3-propylene, 1,2-propylene, 1,3-propylene, 1,4-butanediyl, 1,6-hexanediyl, 1,10-decanediyl, 1,4-cyclohexanediethylene, 2,2'-oxydiethylene, polyoxyethylene, tetraoxyethylene, and the like,

or hydroxyl substituted alkylene such as 2-hydroxymethyl-1,3-propanediyl, 2-hydroxymethyl-2-ethyl-1,3-propanediyl, 2,2-bis(hydroxymethyl)-1,3-propanediyl, and the like.

The barrier layer polymers in accordance with the present invention thus contain planar, electron-deficient aromatic, functionalized bisimide groups in which the aromatic group is preferably a tri- or tetravalent benzene, perylene, naphthalene or anthraquinone nucleus. In addition to the carbonyl groups, aromatic groups in the foregoing structural formulas can have other substituents thereon, such as C<sub>1-6</sub> alkyl, C<sub>1-6</sub>

11

alkoxy, or halogens. Examples of useful imide structures include 1,2,4,5-benzenetetracarboxylic-bisimides:



1,4,5,8-naphthalenetetracarboxylic-bisimides:



3,4,9,10-perylenetetracarboxylic-bisimides:



2,3,6,7-anthraquinonetetracarboxylic-bisimides:



and hexafluoroisopropylidene-2,2',3,3'-benzenetetracarboxylic-bisimides:



12

Especially preferred are those with a fused ring system, such as naphthalenetetracarbonylbisimides and perylenetetracarbonylbisimides, as in many instances they are believed to transport electrons more effectively than a single aromatic ring structure. The preparation of such tetracarbonylbisimides is known and described, for example, in U.S. Pat. No. 5,266,429, the teachings of which are incorporated herein by reference in their entirety. These moieties are especially useful when incorporated into polyester-co-imides as the sole electron-deficient moiety or when incorporated into such polymers in various combinations. The mole percent concentration of the electron deficient moiety in the polymer can desirably range from about 5 mol % to 100 mol %, preferably from about 50 mol % to 100 mol %, with a more preferred range being from about 70 mol % to about 80 mol %.

The barrier layer polymers in accordance with the invention are prepared by condensation of at least one diol compound with at least one dicarboxylic acid, ester, anhydride, chloride or mixtures thereof. Such polymers can have a weight-average molecular weight of 1,500 to 250,000. The preferred polymers of this invention are low molecular weight materials with multiple hydroxyl end groups, and are commonly referred to as polyols. The polyester-co-imide polyols of this invention are prepared by melt polymerization using an excess of hydroxyl functional monomer. Because the hydroxyl sites can function as branch points in the polymer, the ratio of the weight average molecular weight to the number average molecular weight is generally greater than 2, the expected ratio for a linear condensation polymer. Thus the number average molecular weights can be as low as 750, but the weight average molecular weight is much higher for the same molecule. Polyester resin calculations to produce these multifunctional materials are available from Eastman Chemical Company in Kingsport, Tenn. and can be obtained on the world wide web at <http://www.eastman.com/Wizards/ResinCalculationProgram>.

The bisimide structure containing the tetravalent-aromatic nucleus can be incorporated either as a diol or diacid by reaction of the corresponding tetracarbonyldianhydride with the appropriate amino-alcohol or amino-acid. The resulting bisimide-diols or bisimide-diacids may then be polymerized, condensed with diacids or diols, to prepare the barrier layer polymers by techniques well-known in the art, such as interfacial, solution, or melt polycondensation. A preferred technique is melt-phase polycondensation as described by Sorenson and Campbell, in "Preparative Methods of Polymer Chemistry," pp. 113-116 and 62-64, Interscience Publishing, Inc. (1961) New York, N.Y. Preparation of bisimides is also disclosed in U.S. Pat. No. 5,266,429, previously incorporated by reference.

Preferred diacids for preparing the crosslinkable barrier layer polymers include terephthalic acid, isophthalic acid, maleic acid, 2,6-naphthanoic acid, 5-t-butylisophthalic acid, 1,4-cyclohexanedicarboxylic acid, 1,1,3-trimethyl-3-(4-carboxyphenyl)-5-indancarboxylic acid, pyromellitic dianhydride, maleic anhydride, dodecanedioic acid, and methylsuccinic acid.

65 A polymer structure which incorporates the electron deficient naphthalene bisimide as both the acid and the alcohol is shown below as:



f and g represent mole fractions wherein f is from about 0.05 to 0.9 and g is from 0.05 to about 0.9.

A preferred type of monomer is the diacid which comprises a divalent cyclohexyl moiety, such as 1,4-cyclohexanedicarboxylic acid, including both the cis- and trans-isomers thereof. These monomers are commercially available from Eastman Chemical Company of Kingsport, Tenn., and are as a mixture of both the cis- and trans-isomer forms. This type of aliphatic monomer generally provides more desirable electrical properties, such as lower dark decay levels, relative to other aliphatic monomers. The alicyclic moiety also provides an aliphatic moiety in the resulting polymer that is more resistant to degradation than incorporation of a linear aliphatic chain segment. For example, hydrolysis is less of an issue in a coating solution used for extended period of time if cyclohexane dicarboxylic acid rather than sebatic acid makes up the polymer backbone. This has been described in the literature, Ferrar, W. T., Molaire, M. F., Cowdery, J. R., Sorriero, L. J., Weiss, D. S., Hewitt, J. M. Hewitt; Polym. Prepr., 2004, 45(1), 232-233.

A polymer structure which incorporates the electron deficient naphthalene bisimide only as the glycol is shown below as:



m and n represent mole fractions wherein m is from about 0.1 to 0.9 and n is from 0.1 to about 0.9.

Preferred diols and their equivalents for preparing the barrier layer polymers include ethylene glycol, polyethylene glycols, such as tetraethylene glycol, 1,2-propanediol, 2,2'-oxydiethanol, 1,4-butanediol, 1,6-hexanediol, 1,10-decanediol, 1,4-cyclohexanedimethanol, 2,2-dimethyl-1,3-propanediol and 4,4-isopropylidene-bisphenoxy-ethanol. Other

precursors to diols include ethylene carbonate and propylene carbonate.

Although crosslinking can be accomplished through the end groups of the polyester-co-imide, additional crosslinking sites can be incorporated into the polymer through multifunctional monomers. Monomers that contain three and four hydroxyl groups can be introduced during the melt polymerization. These monomers can be used to create branch points in the polymer to change the viscosity characteristics of the polymer. However, the branching can be retarded for the purpose of favoring the functional group incorporation at those positions by making the stoichiometry of the reaction favor the functional group, and by keeping the molecular weight of the polymer low. These differences of branching and functional group incorporation can be readily determined by polymer analysis including size exclusion chromatography and nuclear magnetic resonance (NMR) spectroscopy.

Examples of monomers that are useful for incorporation of crosslinkable acid functional sites into condensation polymers include 1,2,4,5-benzenetetracarboxylic acid (pyromellitic acid), 1,2,4,5-benzenetetracarboxylic dianhydride (py-

romellitic dianhydride), 1,2,3-benzenetricarboxylic acid hydrate (hemimellitic acid), 1,2,4-benzenetricarboxylic acid (trimellitic acid), 1,3,5-benzenetricarboxylic acid (trimesic acid), 1,2,4-benzenetricarboxylic anhydride (trimellitic anhydride). Examples of monomers that can be used to incorporate hydroxy functionality into the polymer include trimethylolpropane, trimethylolpropane ethoxylate, trimethylolethane, pentaerythritol, pentaerythritol ethoxylate,

15

pentaerythritol propoxylate, pentaerythritol propoxylate/ethoxylate, and dimethyl-5-hydroxysisopthalate

Specific structures that incorporate 1,4-cyclohexanedicarboxylic acid, N,N'-Bis-(5-hydroxypentyl)-1,4,5,8-naphthalenetetracarboxylic diimide, 2,2-dimethyl-1,3-propanediol, and trimethylolpropane into the polyester-co-imide are shown below.

wherein a and b are mole fraction of a group and a represents a value between 0.1 and 0.95 and b represents a value between 0.01 and 0.5. More preferably a represents a value between 0.5 and 0.9 and b represents a value between 0.04 and 0.3.

Specific structures that incorporate 1,4-cyclohexanedicarboxylic acid, N,N'-Bis-(5-hydroxypentyl)-1,4,5,8-naphthalenetetracarboxylic diimide, 2,2-dimethyl-1,3-propanediol, and pentaerythritol into the polyester-co-imide are shown below.

16

burgundy solution formed. The contents were then heated to 60 C for 5 hours during which a solid phase separated. The contents were cooled to room temperature and the solid was collected by filtration and washed with methanol. The pink-red solid was recrystallized from dimethylformamide to give 300 g of pink solid, melting point of 210-211 C. m/e 438 in the mass spectrum

The synthesis of Polymer 2 is described below. The syntheses of Polymers 1 and 3-5 are a modification of the Polymer 2 procedure. The amounts of reactants are given in Table 1, and the characterization of the polymer is given in Table 2.

Polymer 2.

Copolymerization of 2,2'-dimethyl-1,3-propanediol, N,N'-Bis-(5-hydroxypentyl)-1,4,5,8-naphthalenetetracarboxylic diimide trimethylolpropane (50/46/4) and 1,4-cyclohexanedicarboxylic acid.



wherein a and b are mole fraction of a group and a represents a value between 0.1 and 0.95 and b represents a value between 0.01 and 0.4. More preferably a represents a value between 0.5 and 0.9 and b represents a value between 0.04 and 0.2.

These and other advantages will be apparent from the detailed description below.

The following examples illustrate the practice of this invention. They are not intended to be exhaustive of all possible variations of the invention. Parts and percentages are by weight unless otherwise indicated.

## EXAMPLES

The invention has been described in detail with particular reference to certain preferred embodiments thereof, but it will be understood that variations and modifications can be effected within the spirit and scope of the invention.

Synthesis of bis(hydroxypentyl)naphthalene bisimide; N,N'-Bis-(5-hydroxypentyl)-1,4,5,8-naphthalenetetracarboxylic diimide A 12 L 3 neck round bottom flask was charged with 1,4,5,8-naphthalenetetracarboxylic dianhydride (260 g, 0.97 mol) and water (5800 mL) and stirred at room temperature for 30 minutes before adding 5-amino-1-pentanol (500 g, 4.85 mol) in a slow stream. The mixture was heated on a steam bath at 3 C until a dark brown

A mixture of 1,4-cyclohexanedicarboxylic acid (CHDA) (106.47 g, 0.618 mol), 2,2'-dimethyl-1,3-propanediol (NPG) (34.05 g, 0.327 mol), trimethylolpropane (TMP) (3.81 g, 0.028 mol), and N,N'-Bis-(5-hydroxypentyl)-1,4,5,8-naphthalenetetracarboxylic diimide (NB5) (155.66 g, 0.355 mol), was charged to a 1 L 3-neck round bottom flask equipped with a steam jacketed column packed with iron filings topped with a distillation head, and an argon inlet tube. The reaction mixture was heated to 220° C. with stirring to produce a transparent, burgundy-colored, homogenous melt. Butylstannic acid (Fascat™ 4100, 0.291 g) was added and the temperature increased to 270° C. over 5 hours. The reaction mixture was stirred overnight. Clear distillate (22 mL) was collected over the course of the reaction. Stirring was stopped, the reaction cooled to room temperature, the polymerization product removed from the reaction vessel and submitted for assay. The glass transition temperature, molecular weight, acid number and hydroxyl number were determined. The results are given in Table 2.

Polymer 6.

Copolymerization of 2,2'-dimethyl-1,3-propane diol, N,N'-Bis-(5-hydroxypentyl)-1,4,5,8-naphthalenetetracarboxylic diimide, -pentaerythritol (75/17/8) and 1,4-cyclohexanedicarboxylic acid.

A mixture of cyclohexanedicarboxylic acid (CHDA) (86.59 g, 0.503 mol), 2,2'-dimethyl-1,3-propanediol (NPG)

(10.57 g, 0.102 mol), pentaerythritol (PER) (6.50 g, 0.048 mol), and N,N'-Bis-(5-hydroxypentyl)-1,4,5,8-naphthalene-tetracarboxylic diimide (NB5) (196.33 g, 0.448 mol), was charged to a 1 L 3-neck round bottom flask equipped with a steam jacketed column packed with iron filings topped with a distillation head, and an argon inlet tube. The reaction mixture was heated to 220° C. with stirring to produce a transparent, burgundy-colored, homogenous melt. Butylstannoic acid (Fascat™ 4100, 0.15 g) was added and the temperature increased to 260° C. over 5 hours. Clear distillate (16 mL) was collected over the course of the reaction. Stirring was stopped, the reaction mixture cooled to room temperature, the polymerization product removed from the reaction vessel and submitted for assay. The glass transition temperature, molecular weight, acid number and hydroxyl number were determined. The results are given in Table 2.

TABLE 1

| .Synthesis of Polymers 1-5 |                        |                       |                      |                        |
|----------------------------|------------------------|-----------------------|----------------------|------------------------|
| Polymer                    | CHDA                   | NPG                   | TMP                  | NB5                    |
| 1                          | 106.80 g,<br>0.620 mol | 37.11 g,<br>0.356 mol | —                    | 156.08 g,<br>0.356 mol |
| 2                          | 106.47 g,<br>0.618 mol | 34.05 g,<br>0.327 mol | 3.81 g,<br>0.028 mol | 155.66 g,<br>0.355 mol |
| 3                          | 89.87 g,<br>0.522 mol  | 12.83 g,<br>0.123 mol | 8.26 g,<br>0.062 mol | 189.04 g,<br>0.431 mol |
| 4                          | 86.66 g,<br>0.503 mol  | 10.57 g,<br>0.102 mol | 6.41 g,<br>0.048 mol | 196.36 g,<br>0.448 mol |
| 5                          | 86.96 g,<br>0.505 mol  | 13.10 g,<br>0.126 mol | 3.21 g,<br>0.024 mol | 196.72 g,<br>0.449 mol |

TABLE 2

| Characterization of Polymers 1-6 |                |                |                |                                |                                       |                                |
|----------------------------------|----------------|----------------|----------------|--------------------------------|---------------------------------------|--------------------------------|
| Polymer                          | T <sub>g</sub> | M <sub>n</sub> | M <sub>w</sub> | M <sub>w</sub> /M <sub>n</sub> | Hydroxy Concentration (meq/g polymer) | Acid Number (mg KOH/g polymer) |
| 1                                | 72             | 8120           | 56500          | 7                              | 2.26                                  | 4.5                            |
| 2                                | 55             | 4860           | 12300          | 2.5                            | 0.65                                  | 3.6                            |
| 3                                | 84             | 6140           | 43100          | 7                              | 0.4                                   | 6.1                            |
| 4                                | 75             | 5700           | 40000          | 7                              | 0.38                                  | 4.7                            |
| 5                                | 89             | 9370           | 64100          | 6.8                            | 0.26                                  | 4.1                            |
| 6                                | 82             | 4010           | 15000          | 3.7                            | 0.9                                   | 3.1                            |

M<sub>n</sub> and M<sub>w</sub> were obtained by size-exclusion chromatography (SEC) in 1,1,1,3,3,3-hexafluoroisopropanol (HFIP) containing 0.01M tetraethylammonium nitrate using two 7.5 mm×300 mm PLgel mixed-C columns. Polymethylmethacrylate equivalent molecular weight distributions are reported for the samples.

<sup>19</sup>F NMR Hydroxyl Concentration analysis was performed in replicate, with separate sample preparations. The <sup>19</sup>F NMR analyses were performed at an observe frequency of 282.821 MHz, ambient temperature, and CDCl<sub>3</sub> was the solvent. The samples were derivatized with trifluoroacetylimidazole (TFAI), which converts the hydroxyl groups to fluorinated ester groups. Trifluorotoluene (TFT) was used as an internal reference, thus allowing quantification by <sup>19</sup>F NMR spectroscopy.

Acid numbers were obtained by dissolving the polymer in 50/1 MeCl<sub>2</sub>/MeOH and titration to a potentiometric end point with hexadecyltrimethylammonium hydroxide (HDTMAH). The acid number is based on the carboxylic acid end point is 7.1.

## Example 1

The hydroxyl equivalent weight of polymer 4 (0.38 meq/mole of hydroxyl group) was calculated at 2632 grams. The NCO equivalent wt of the Trixene B7963 (including solvent) is reported at 681 grams by the manufacturer. This information was used to mix formulation 1 at a 1:1 polymer 6 to the Trixene B7963 diethyl malonate blocked isocyanate. A 40% excess hydroxyl was provided by the high molecular weight, hydroxyl-functional, partially hydrolyzed vinyl chloride/vinyl acetate resin UCAR (trademark) VAGH, obtained from Dow chemical. The materials were dissolved in 1,1,2 trichloroethane at a dilution appropriate for dip coating the appropriate thickness for the experiment. Dibutyl tin dilaurate from Aldrich Chemicals was used as a catalyst at 0.40 wt %.

| Formulation 1 |                   |                        |      |                     |                          |
|---------------|-------------------|------------------------|------|---------------------|--------------------------|
|               | NCO Equivalent Wt | Hydroxyl Equivalent Wt | Gram | NCO Equivalent mole | Hydroxyl Equivalent mole |
| Polymer 4     |                   | 2632                   | 218  |                     | 0.083                    |
| Trixene B7963 | 681               |                        | 57   | 0.084               | 1.01                     |
| VAGH          |                   | 951                    | 32   |                     | 0.034                    |
|               |                   |                        |      | TOTAL               | 0.40                     |

Formulation 1 was dip coated over a nickel sleeve pre-coated with six microns surface smoothing layer as described in Molaire U.S. Patent Publication Ser. No. 2006/0009563 entitled "Aqueous Metal oxide Composition for Dip Coating and Electrophotographic Application". The barrier layer was then cured in a Blue M oven by the following conditions. The oven temperature was ramped to 170° C within 30 minutes. The temperature was kept at 170° C. for one hour. The sleeves were cooled down temperature over 30-minute period the sleeve substrate was weighted before and after coating the barrier layer formulation. The information was used to estimate an average coverage of the barrier layer on the sleeve. The results are shown on Table 3.

The barrier layer coated sleeves were then dip coated in the charge generation layer dispersion of Molaire & Al, U.S. Patent Publication No. 2005/0266330, entitled "Newtonian Ultrasonic Insensitive Charge Generating Layer Dispersion Composition And a Method for Producing the Composition". The charge generation dispersion utilizes the same 1,1,2-trichloroethane solvent used to coat the baffle layer. The sleeve was weighed again after the CGL coating. As seen in Table 2 a positive thickness growth indicates that the cross-linked barrier was not adversely attacked by the solvent.

TABLE 3

|       | BL mm/s | BL g/ft <sup>2</sup> | CGL mm/s | CGL g/ft <sup>2</sup> | BL + CGL |
|-------|---------|----------------------|----------|-----------------------|----------|
| Ctg 1 | 0.6     | 0.11                 | 0.6      | 0.01                  | 0.124    |
| Ctg 2 | 0.6     | 0.09                 | 1        | 0.04                  | 0.127    |
| Ctg 3 | 1.5     | 0.15                 | 0.6      | 0.01                  | 0.156    |
| Ctg 4 | 1.5     | 0.13                 | 1.2      | 0.05                  | 0.174    |

BL is Barrier Layer  
CGL is Charge Generation Layer

## Comparative Example 1

A barrier composition similar to formulation 1 was assembled, except that an excess hydroxyl equivalent was provided by a pentaerythritol ethoxylate (3/4 EO/OH) oligomer, obtained from Aldrich Chemicals. The excess hydroxyl equivalent was 130%. Comparative formulation 1 was coated using the same procedure as in example 1. As can be seen from Table 4, thickness erosion is measured after the CGL coating, suggesting detrimental attack of the barrier layer. The imbalance in the OH/NCO is enough to prevent efficient cross-linking, illustrating the importance of stoichiometry for the cross-linking process.

## Comparative Formula 1

|           | NCO<br>Equiv-<br>alent<br>Wt | Hydroxyl<br>Equivalent<br>Wt | Gram | NCO<br>Equiv-<br>alent<br>mole | Hydroxyl<br>Equivalent<br>mole | Equivalent<br>Ratio<br>OH/NCO |
|-----------|------------------------------|------------------------------|------|--------------------------------|--------------------------------|-------------------------------|
| Polymer 4 | 2632                         | 218                          |      | 0.083                          | 0.99                           |                               |
| Trixene   |                              |                              |      | 0.084                          |                                |                               |
| B7963     | 681                          |                              | 57   |                                | 1.01                           |                               |
| PET 3/4   |                              | 101.3                        | 11   |                                | 0.109                          | 1.30                          |
|           |                              |                              |      | TOTAL                          | 2.29                           |                               |

TABLE 4

|       | BL<br>m/s | BL<br>g/ft <sup>2</sup> | CGL<br>mm/s | CGL<br>g/ft <sup>2</sup> | Actual<br>BL + CG Wt |
|-------|-----------|-------------------------|-------------|--------------------------|----------------------|
| Ctg 5 | 0.6       | 0.13                    | 0.8         | -0.028                   | 0.102                |
| Ctg 6 | 1         | 0.126                   | 0.8         | -0.045                   | 0.081                |
| Ctg 7 | 1.5       | 0.179                   | 0.8         | -0.053                   | 0.126                |
| Ctg 8 | 2         | 0.179                   | 0.8         | -0.049                   | 0.130                |

BL is Barrier Layer

CGL is Charge Generation Layer

## Example 2

Formulation 2, using polymer 5 (hydroxyl equivalent wt, calculated at 3846) was coated on nickel sleeve, following the procedure of example 1. The coated sleeves were evaluated for sensitometry and image quality in a Nexpress 2100 Digital printer at three different environmental conditions. The toe voltages and the overall breakdown numbers are shown in Table 5.

|           | Formulation 2                |                              |      |                                |                                |                               |
|-----------|------------------------------|------------------------------|------|--------------------------------|--------------------------------|-------------------------------|
|           | NCO<br>Equiv-<br>alent<br>Wt | Hydroxyl<br>Equivalent<br>Wt | Gram | NCO<br>Equiv-<br>alent<br>mole | Hydroxyl<br>Equivalent<br>mole | Equivalent<br>Ratio<br>OH/NCO |
| Polymer 5 | 3846                         | 198                          |      | 0.053                          | 0.85                           |                               |
| Trixene   |                              |                              |      |                                |                                |                               |
| B7963     | 681                          |                              | 43   | 0.063                          |                                | 1.18                          |
| VAGH      |                              | 951                          | 34   |                                | 0.036                          | 0.57                          |
|           |                              |                              |      | TOTAL                          | 1.41                           |                               |

TABLE 5

| 5      | Barrier<br>g/ft <sup>2</sup> | Toe<br>Voltage @<br>75 F./30%<br>RH | Toe<br>Voltage @<br>75 F./30%<br>RH | Toe<br>Voltage @<br>78 F./81%<br>RH | Breakdown<br># |
|--------|------------------------------|-------------------------------------|-------------------------------------|-------------------------------------|----------------|
|        |                              |                                     |                                     |                                     |                |
| Ctg 9  | 0.03                         | 79                                  | 93                                  | 77                                  | 2.4            |
| Ctg 10 | 0.07                         | 91                                  | 114                                 | 68                                  | 2.1            |

15

## Example 3

Formulation 3, using polymer 6 (1111 hydroxyl equivalent wt) exclusively, provided a 60% excess hydroxyl equivalent.

20 Nickel sleeves were coated using the procedure of Example 1.

Formulation 3

|           | NCO<br>Equiv-<br>alent<br>Wt | Hydroxyl<br>Equivalent<br>Wt | Gram | NCO<br>Equiv-<br>alent<br>mole | Hydroxyl<br>Equivalent<br>mole | Equivalent<br>Ratio<br>OH/NCO |
|-----------|------------------------------|------------------------------|------|--------------------------------|--------------------------------|-------------------------------|
| polymer 6 |                              | 1111                         | 199  |                                | 0.179                          | 1.61                          |
| Trixene   |                              |                              |      | 0.110                          |                                |                               |
| B7963     | 681                          |                              | 75   |                                |                                | 0.62                          |
| VAGH      |                              | 951                          | 0    |                                | 0.000                          | 0.00                          |
|           |                              |                              |      | TOTAL                          | 1.61                           |                               |

35

The sleeves were evaluated in a Nexpress 21000 digital printer @ 7F/30% RH. The toe voltages are shown in Table 6

40

TABLE 6

|        | Barrier Layer<br>g/ft <sup>2</sup> | CGL g/ft <sup>2</sup> | Residual Voltage @ 75 F./30% RH |
|--------|------------------------------------|-----------------------|---------------------------------|
| Ctg 11 | 0.04                               | 0.02                  | 89                              |
| Ctg 12 | 0.05                               | 0.02                  | 113                             |
| Ctg 13 | 0.06                               | 0.03                  | 115                             |

50

## Example 4

Formulation 3 was further coated at various thicknesses on bare aluminum drums. The drums were evaluated for breakdown on the Nexpress 2100 digital printer. The results are shown on Table 7.

55

TABLE 7

|        | Barrier Layer<br>g/ft <sup>2</sup> | CGL OD | Breakdown # |
|--------|------------------------------------|--------|-------------|
| Ctg 14 | 0                                  | 0.57   | 18          |
| Ctg 15 | 0.07                               | 0.57   | 3.9         |
| Ctg 16 | 0.09                               | 0.57   | 2.6         |
| Ctg 17 | 0.13                               | 0.57   | 2.9         |
| Ctg 18 | 0.2                                | 0.57   | 2.3         |

60

CGL is Charger Generation Layer

## 21

The invention has been described in detail with particular reference to certain preferred embodiments thereof, but it will be understood that variations and modifications can be effected within the spirit and scope of the invention.

The invention claimed is:

1. A photoconductive element comprising an electrically conductive support, an electrical barrier layer disposed over said electrically conductive support, a charge generation layer capable of generating positive charge carriers when exposed to actinic radiation disposed over said barrier layer, said barrier layer comprising a crosslinker, and a crosslinkable condensation polymer having covalently bonded as repeating units in the polymer chain, aromatic tetracarbonyl-bisimide groups of the formula:



wherein Ar represents a tetravalent aromatic group.

2. The photoconductive element of claim 1 wherein said crosslinker comprises diethyl malonate blocked isocyanate.

3. The photoconductive element of claim 2 wherein said crosslinking agent comprises:



R = (CH<sub>2</sub>)<sub>6</sub>

4. The photoconductive element of claim 3 wherein said crosslinking agent contains a catalyst.

5. The photoconductive element of claim 1 wherein the electrically conductive support comprises a flexible material having a layer of metal disposed thereon.

6. The photoconductive element of claim 5 wherein the metal is nickel.

## 22

7. The photoconductive element of claim 5 wherein the metal is aluminum.

8. The photoconductive element of claim 1 wherein the barrier layer has a thickness of between 0.5 and 3 micrometers.

10 9. A photoconductive element comprising an electrically conductive support, an electrical barrier layer disposed over said electrically conductive support, a charge generation layer capable of generating positive charge carriers when exposed to actinic radiation disposed over said barrier layer, said barrier layer comprising a crosslinker, and a condensation polymer, which polymer comprises a crosslinkable poly-15 ester-co-imide that contains an aromatic tetracarbonyl-bisimide group and has the formula:



where

x is the mole fraction of tetracarbonyl-bisimide diacid residue due in the diacid component of the monomer feed,

y is the mole fraction of tetracarbonyl-bisimide glycol residue due in the glycol component of the monomer feed, and such that x+(1-y)=0.1 to 1.9;

Ar¹ and Ar² are tetravalent aromatic groups having from 6 to 20 carbon atoms and may be the same or different;

R¹, R², R³, and R⁴ are alkylene and may be the same or different;

R⁵ is alkylene or arylene; and

R⁶ is alkylene.

10 10. A photoconductive element comprising an electrically conductive support, an electrical barrier layer disposed over said electrically conductive support, a charge generation layer capable of generating positive charge carriers when exposed to actinic radiation disposed over said barrier layer, said barrier layer comprising a crosslinker, and a condensation polymer derived from the formula:



f and g represent mole fractions wherein f is from about 0.05 to 0.9 and g is from 0.05 to about 0.9.

**11.** A photoconductive element comprising an electrically conductive support, an electrical barrier layer disposed over said electrically conductive support, a charge generation layer capable of generating positive charge carriers when exposed to actinic radiation disposed over said barrier layer, said barrier layer comprising a crosslinker, and a condensation polymer, comprising a condensation polymer having covalently bonded as repeating units in the polymer chain, aromatic tetracarbonylbisimide groups derived from the formula:

wherein a and b are mole fraction of a group and a represents a value between 0.1 and 0.95 and b represents a value between 0.01 and 0.4.

**12.** A method of forming an image comprising providing a photoreceptor, charging said photoreceptor, exposing said photoreceptor to actinic radiation, developing said image with a toner, and transferring said image to a receiver sheet, wherein the photoreceptor comprises an electrically conductive support, an electrical barrier layer disposed over said electrically conductive support, a charge generation layer capable of generating positive charge carriers when exposed to actinic radiation disposed over said barrier layer, said barrier layer comprising a crosslinker, and a condensation polymer comprising a crosslinkable condensation polymer having



25

covalently bonded as repeating units in the polymer chain, aromatic tetracarbonylbisimide groups of the formula:



5

10

wherein Ar represents a tetravalent aromatic group.

13. A method of forming an image comprising providing a photoreceptor, charging said photoreceptor, exposing said photoreceptor to actinic radiation, developing said image with a toner, and transferring said image to a receiver sheet, wherein the photoreceptor comprises an electrically conductive support, an electrical baffle layer disposed over said electrically conductive support, a charge generation layer capable of generating positive charge carriers when exposed to actinic radiation disposed over said barrier layer, said barrier layer comprising a crosslinker, and a condensation polymer comprises a crosslinkable polyester-co-imide that contains an aromatic tetracarbonylbisimide group and has the formula:



15

20

25

30

26

-continued



where

x is the mole fraction of tetracarbonylbisimide diacid residue in the diacid component of the monomer feed,

y is the mole fraction of tetracarbonylbisimide glycol residue in the glycol component of the monomer feed, and such that  $x=(1-y)=0.1$  to  $1.9$ ;

$Ar^1$  and  $Ar^2$  are tetravalent aromatic groups having from 6 to 20 carbon atoms and may be the same or different.

$R^1$ ,  $R^2$ ,  $R^3$ , and  $R^4$  are alkylene and may be the same or different;

$R^5$  is alkylene or arylene;

$R^6$  is alkylene.

\* \* \* \* \*

UNITED STATES PATENT AND TRADEMARK OFFICE  
**CERTIFICATE OF CORRECTION**

PATENT NO. : 7,541,124 B2  
APPLICATION NO. : 11/210100  
DATED : June 2, 2009  
INVENTOR(S) : Michel F. Molaire et al.

Page 1 of 1

It is certified that error appears in the above-identified patent and that said Letters Patent is hereby corrected as shown below:

Cover Page of Patent, OTHER PUBLICATIONS:  
delete "Michel Molair" and insert -- Michel Molaire --.

Cover Page of Patent, OTHER PUBLICATIONS:  
delete "Barier" and insert -- Barrier --.

Column 25, claim 13, line 18, after "support, an electrical" delete "baffler"  
and insert -- barrier --.

Column 26, claim 13, line 25, after "such that" delete "x = (1-y) = 0.1 to 1.9"  
and insert -- x + (1-y) = 0.1 to 1.9 --.

Column 26, claim 13, line 27, after "atoms and may be the same or" delete  
"different." and insert -- different: --.

Signed and Sealed this

Eighteenth Day of August, 2009



David J. Kappos  
*Director of the United States Patent and Trademark Office*